

## UNITED STATES PATENT OFFICE

2,666,744

## SULFURIZED GREASE COMPOSITIONS

Joseph A. Dixon, Berkeley, Calif., assignor to  
California Research Corporation, San Francisco, Calif., a corporation of Delaware

No Drawing. Application March 5, 1952,  
Serial No. 275,027

16 Claims. (Cl. 252—33.6)

1

This invention pertains to grease compositions containing sulfurized metal soap grease thickening agents (e. g., sulfurized sodium oleate).

Industrial engineers are constantly striving to improve upon engineering performance and to incorporate new materials, new techniques, etc. into the various industries. For example, in the automotive industry, there is the desire to manufacture smaller internal combustion engines without sacrificing power output. In fact, many of these smaller engines are designed to deliver greater power than their larger counterparts. The same smaller engines have considerably less bearing surfaces than their larger predecessors, which means that the bearings bear greater loads than before.

Similarly, the continuing trend to manufacture automobiles with lower centers of gravity has made it necessary to use smaller and smaller gears, particularly in such gear assemblies as the differentials and transmissions. The smaller gears thus used also have considerably greater pressures exerted upon them per unit area than the older type large gear assemblies. The higher loads on bearings and gears demand better compounding agents in grease compositions.

For quite some period of time, sulfur has been used in lubricating oil compositions for such purposes as, for example, to impart extreme pressure (E. P.) characteristics, anti-wear characteristics, oxidation inhibiting characteristics, etc., to the lubricant. This sulfur has been obtained from free sulfur, thioethers, mercaptans, mercaptides, etc. However, sulfur compounds which are presently used in lubricants for such purposes are known to be corrosive and to promote wear, particularly to steel and copper surfaces. Thus, it has been necessary to add secondary additives for the specific purpose of inhibiting this corrosiveness caused by the sulfur compounds.

It is, therefore, an object of this invention to prepare grease compositions containing sulfur compounds as extreme pressure agents, which sulfur compounds are not corrosive to steel.

It is a further object of this invention to prepare grease compositions having extreme pressure characteristics, anti-wear characteristics, etc., without the use of secondary additives to inhibit corrosion to metals, such as steel and copper, or to inhibit bleeding.

These and further objects of this invention will be apparent from the following description and the appended claims.

According to this invention, it has been discovered that, unexpectedly, grease compositions

2

thickened by metal soaps sulfurized to a critical degree have greatly enhanced anti-wear characteristics while simultaneously being relatively non-corrosive. The grease compositions of this invention comprise lubricating oils and sulfurized metal soaps.

The use of the term "sulfurizing" herein means the reaction of sulfur with the metal soap thickening agent as described hereinbelow.

10 In the grease compositions of this invention, metal soaps which thicken lubricating oils to the consistency of greases are sulfurized. These sulfurized metal soaps are metal soaps of fatty acids having from 1 to 3 double bonds per fatty acid anion. It is preferred that the fatty acid anions contain only 1 double bond. When using fatty acid anions containing 2 or 3 double bonds, it is beneficial to use, in addition, small amounts of fatty acids containing only 1 double bond or 20 no double bonds.

25 The unsaturated fatty acids which are used in the formation of the soaps include the straight or branched-chain, unsaturated fatty acids containing from 9 to 30 carbon atoms.

30 Examples of unsaturated fatty acids which can be used in the formation of the sulfurized metal soap grease thickening agents according to this invention include undecylenic acid, myristoleic acid, palmitoleic acid, oleic, erucic acid, brassidic acid, cetoleic acid, linolenic acid, linolinic acid, etc.

35 The metals which can be used in the formation of the soaps include the metals of groups I, II and III of Mendeleef's periodic table. Particular metals include lithium, sodium, potassium, magnesium, calcium, zinc, strontium, cadmium, barium and aluminum.

40 Although sulfurization seems to be limited to the soaps of unsaturated fatty acids, it is not intended that the grease composition should contain only the soaps of unsaturated fatty acids. Soaps of mixtures of saturated and unsaturated fatty acids may be used in the grease compositions of this invention. However, the soaps of 45 saturated fatty acids do not appear to enter into the sulfurization reaction.

45 The sulfur is present in an amount of from about 0.25 to 1.0 atom of sulfur per double bond of the unsaturated fatty acid. In other words, 50 in the average, the unsaturated soap molecule contains from about 0.25 to 1.0 atom of sulfur for each double bond present, or evaluated as such by the iodine number of the unsaturated soaps. The value of one atom of sulfur per double bond is critical, because when its value ex-

ceeds one, the resulting grease composition has a tendency to bleed, and, also, the grease deteriorates rapidly.

Suitable base oils include a wide variety of lubricating oils such as naphthenic base, paraffin base, and mixed base mineral oils, other hydrocarbon lubricants, e. g., lubricating oils derived from coal products, and synthetic oils, e. g., alkylene polymers (such as polymers of propylene, butylene, etc., and mixtures thereof), alkylene oxide type polymers, dicarboxylic acid esters, liquid esters of acids of phosphorus and silicon, alkyl benzene polymers, polysiloxanes, etc. Synthetic oils of the alkylene oxide type polymers which may be used include those exemplified by the alkylene oxide polymers (e. g., propylene oxide polymers) and derivatives, including alkylene oxide polymers prepared by polymerizing alkylene oxides, e. g., propylene oxide, in the presence of water or alcohols, e. g., ethyl alcohol, and esters of alkylene oxide type polymers, e. g., acetylated propylene oxide polymers prepared by acetylating propylene oxide polymers containing hydroxyl groups.

Synthetic oils of the dicarboxylic acid ester type include those which are prepared by esterifying such dicarboxylic acids as adipic acid, azaleic acid, suberic acid, sebacic acid, alkenyl succinic acid, fumaric acid, maleic acid, etc., with alcohols such as butyl alcohol, hexyl alcohol 2-ethylhexyl alcohol, dodecyl alcohol, etc. Examples of dicarboxylic acid ester synthetic oils include dibutyl adipate, dihexyl adipate, di-2-ethylhexyl sebacate, di-n-hexyl fumaric polymers, etc.

Synthetic oils of the alkyl benzene type include those which are prepared by alkylating benzene (e. g., dodecyl benzene, tetradecyl benzene, etc.).

Synthetic oils of the type of liquid esters of acids of phosphorus include the esters of phosphoric acid, e. g., tricresyl phosphate; the esters of phosphonic acid, e. g., diethyl ester of decane phosphonic acid, etc.

Synthetic oils of the type of the liquid esters of silicon and polysiloxanes include those exemplified by tetra (2-ethylhexyl) silicate, hexa (4-methyl-2-pentoxy) disiloxane, tetra (4-methyl-2-pentyl) silicate, tetra (1,3-dimethylbutyl) silicate, poly-methyl phenyl siloxane, polymethyl siloxane, etc.

Although, as stated hereinabove, the amount of sulfur present in the metal soap thickening agents can be from about 0.25 to about 1.0 atom of sulfur per double bond of the unsaturated fatty acid anion, the preferred amount of sulfur present in the metal soap thickening agent of grease compositions can vary with the metal of the soap. For example, in a grease composition thickened with calcium soaps, it is preferred to use sulfur in an amount of 0.3 to 0.5 atom of sulfur per double bond in the unsaturated fatty acid anion of the soap; and for a grease composition thickened by lithium, sodium or potassium soaps, for example, it is preferred to use from 0.7 to 0.95 atom of sulfur per double bond of the fatty acid anion of the soap.

It is understood that the amount of soap used in the grease compositions of this invention is that amount which will thicken the base oil to the consistency of a grease. Although amounts of about 3% by weight to about 50% by weight can be used, it is preferred to use from about 10% to 25%.

Methods of preparing grease compositions of this invention include the following:

1. Forming a metal soap from an unsaturated fatty acid, or a mixture of fatty acids containing unsaturated fatty acids, then heating the soap (i. e., the soap itself or a solution or dispersion of the soap in oil) thus formed with sulfur in an amount such that the sulfurized soap contains from 0.25 to 1.0 atom of sulfur per double bond of fatty acid anion, then forming the grease therefrom by adding the proper amount of oil.

2. Reacting sulfur with a grease composition comprising a lubricating oil thickened by a metal soap of an unsaturated fatty acid, etc.

The reaction of the sulfur and the soaps of unsaturated fatty acids can be accomplished at temperatures between 225° F. and 600° F. The period of time required for the reaction depends on the temperature at which the reaction is accomplished and the amount of sulfur which is to be incorporated into the soap. The higher the temperature, the less the reaction time necessary for the completion of the reaction.

The exact nature of the reaction between the sulfur and the soaps of the unsaturated fatty acids is not known. It is not known in what manner the sulfur combines with the metal soaps. The degree of unsaturation of the fatty acid remains practically the same after the reaction with the sulfur as before the reaction; that is, the iodine number of the fatty acid is practically the same after the reaction with the sulfur as before. It is fairly well established that the reaction of sulfur with the metal soap is not accomplished at the expense of the double bond of the fatty acid anion.

As stated hereinabove, the soap thickening agents may also contain soaps of saturated fatty acids. It is preferred that the soaps of unsaturated fatty acids are present in amounts of more than 15% of the total amount of fatty acids.

However, when the amount of sulfur present is about one atom of sulfur per double bond, the total amount of unsaturated fatty acid anion may be only 5% of the total amount of fatty acid anions.

The use of the sulfurized metal soaps in grease compositions according to this invention enhances extreme pressure characteristics, anti-wear characteristics, etc., but still the grease compositions of this invention are non-corrosive to copper and steel. Furthermore, the grease compositions of this invention have greater resistance to oxidation, greater resistance to bleeding, and have a better texture than greases thickened with unsulfurized soaps.

The grease compositions sulfurized according to the present invention can be prepared by methods exemplified by the following:

#### EXAMPLE 1.—PREPARATION OF A SULFURIZED LITHIUM SOAP GREASE

A mixture of 28.2 grams (0.1 equivalent) of highly refined oleic acid, 28.4 grams (0.1 equivalent) of stearic acid and 391 grams of a California solvent-refined paraffin base petroleum oil having a viscosity of 185 SSU at 210° F., was heated with stirring to 170° F., at which temperature the acids were neutralized by 100 ml. of 2N lithium hydroxide solution. This whole mixture was heated with stirring to 400° F., at which temperature 3.2 grams of sulfur was added. After the reaction mixture had been heated at a temperature ranging from 410 to 420° F. for two hours, the product was cooled in a large evaporating dish.

EXAMPLE 2.—PREPARATION OF A SULFURIZED SODIUM  
SOAP GREASE.

An aqueous solution of 4.0 grams (0.1 equivalent) of sodium hydroxide was added to a mixture of 14.2 grams (0.05 equivalent) of stearic acid, 14.1 grams (0.05 equivalent) of oleic acid, and 76.5 grams of California solvent-refined paraffin base oil having a viscosity of 480 SSU at 100° F. This mixture was heated with stirring to 430° F., and sufficient stearic acid was added to adjust the pH to 7.0. The solution was cooled in an evaporating dish, resulting in the formation of a pale brown, smooth, soft grease. To this grease was added 1.3 grams of sulfur, and the mixture was heated with stirring to 400° F. for 1 hour. The resulting product was a very soft, smooth grease containing 0.82% sulfur.

EXAMPLE 3.—PREPARATION OF SULFURIZED SODIUM  
SOAP GREASE

An aqueous solution of 4.0 grams (0.1 equivalent) of sodium hydroxide was added to a mixture of 14.2 grams (0.05 equivalent) of stearic acid, 14.1 grams (0.05 equivalent) of oleic acid, 25 and 76.5 grams of California solvent-refined paraffin base oil having a viscosity of 480 SSU at 100° F. This mixture was heated with stirring to 430° F., and sufficient stearic acid was added to adjust the pH to 7.0. The solution was cooled 30 in an evaporating dish, resulting in the formation of a pale brown, smooth, soft grease. To this grease was added 1.3 grams of sulfur, and the mixture was heated at 250° F. for 24 hours. The resulting product was a soft, smooth grease. 35

The resulting product was a soft, smooth grease. 35

number=52), 610 grams of hydrated lime, 2000 grams of a California solvent-refined paraffin base oil having a viscosity of 450 SSU at 100° F. and 500 ml. of water was heated at 300° F. for one hour in a grease kettle at an absolute pressure of about 65 pounds per square inch. After the temperature had been reduced to 200° F. and the pressure reduced to atmospheric pressure, sufficient stearic acid was added so that the mixture had a content of about 0.1% free fatty acid. The whole mixture was heated to 300° F., at which temperature 200 grams of sulfur was added, and the sulfurization reaction was continued at 300° F. for 3 hours. After the mixture had been cooled, 6500 grams of the above petroleum oil was added, and the grease was hydrated by the addition of 425 ml. of water at a temperature of 235° F., which cooled the grease to 215° F. An additional amount of 11,200 grams of a California solvent-refined paraffin base petroleum oil having a viscosity of 140 SSU at 210° F. was added. The resulting grease had a melting point of 212° F., an unworked penetration of 321 and a worked penetration of 355 (60 strokes).

The following Table I presents reaction conditions, inspections and general data on sulfurized metal soap greases of this invention. Base oil "A" was a California solvent-refined paraffin base oil having a viscosity of 185 SSU at 210° F.; base oil "B" was a California solvent-refined paraffin base oil having a viscosity of 480 SSU at 100° F.; and base oil "C" was a California solvent-refined paraffin base oil having a viscosity of 450 SSU at 100° F.

TABLE I

*Reaction conditions and properties of sulfurized metal soap greases*

| Test No. | Soap (percent by weight) | Base oil | Sulfurization reaction                                  |             |             | Percent sulfur in grease | ASTM dropping point | Penetration |                     |
|----------|--------------------------|----------|---------------------------------------------------------|-------------|-------------|--------------------------|---------------------|-------------|---------------------|
|          |                          |          | Sulfur (gm. atoms/mole of unsaturated fatty acid anion) | Temp. (°F.) | Time (hrs.) |                          |                     | Worked      | Unworked 60 strokes |
| 12-C     | 110.0                    | A        | 0.0                                                     |             |             |                          | 376                 | 234         | 279                 |
| 12-CS    | 110.0                    | A        | 0.5                                                     | 400         |             |                          | 388                 | 305         | 286                 |
| 15-2S    | 110.4                    | A        | 0.5                                                     | 250         | 24          | 0.71                     | 400+                | 261         | 330                 |
| 15-3S    | 110.4                    | A        | 0.5                                                     | 400         | 1           | 0.51                     | 402                 | 260         | 307                 |
| 22-A     | 114.0                    | A        | 0.0                                                     |             |             |                          | 382                 |             |                     |
| 22-B     | 114.0                    | A        | 0.9                                                     | 400         | 1           | 0.70                     | 389                 | 203         | 260                 |
| 22-C     | 114.0                    | A        | 0.9                                                     | 250         | 24          | 0.96                     | 393                 | 216         | 267                 |
| 23-C     | 226.8                    | B        | 0.9                                                     | 400         | 1           | 0.82                     | 366                 | 305         | 331                 |
| 23-A     | 226.8                    | B        | 0.0                                                     |             |             |                          | 364                 | 290         | 332                 |
| 45-A     | 320.0                    | C        | 0.0                                                     |             |             |                          | 206                 | 183         | 207                 |
| 42-A     | 320.0                    | C        | 0.9                                                     | 300         | 2           | 0.87                     | 348                 | 370         |                     |

<sup>1</sup> Equal parts by weight of lithium oleate and lithium stearate.

<sup>2</sup> Equal parts by weight of sodium oleate and sodium stearate.

<sup>3</sup> Calcium soap of a tallow having an iodine number of 52.

EXAMPLE 4.—PREPARATION OF A LITHIUM SOAP  
GREASE

A mixture of 85.4 grams (0.3 equivalent) of oleic acid, 1000 grams of a California solvent-refined paraffin base oil, 12.6 grams (0.3 equivalent) of lithium hydroxide monohydrate and 100 ml. of water was heated to 400° F. When the mixture cooled, a fibrous, pale yellow grease was obtained. To this grease was added 8.64 grams (0.27 gram atoms) of sulfur, and the heating was continued at 400° F. for one hour. After milling, the dark, reddish brown, buttery grease contained 1.40% sulfur.

EXAMPLE 5.—PREPARATION OF A CALCIUM SOAP  
GREASE

A mixture of 4000 grams of tallow (iodine 75 mixture of California solvent-refined paraffin

The data presented hereinbelow in Table II show the effectiveness of sulfurized metal soap thickening agents in reducing wear and in increasing the extreme pressure properties of greases, comparisons being made with greases prepared from unsulfurized metal soap thickening agents. The soap used was a calcium soap of a tallow having an iodine number of 52. The sulfurization reaction was accomplished at 300° F. for a period of 2 hours. The Timken and Almen tests are described in "Lubricants and Lubrication" by Clower, published by McGraw-Hill Book Company in 1939, pages 145 to 148, inclusive. The Falex tests are described in the "Journal of the Institute of Petroleum," vol. 32, April 1946. In the following table, base oil "D" was a mixture of California solvent-refined paraffin

base oil having a viscosity of 185 SSU at 210° F. and a California solvent-refined base oil having a viscosity of 450 SSU at 100° F. Base oil "C" was the same as described in connection with Table I.

TABLE II  
*Reaction conditions and wear characteristics of sulfurized metal soap greases*

| Test No. | Soap (percent by weight) | Base oil | Sulfurization reaction-Sulfur (gm. atoms/mole of unsaturated fatty acid: anion) | Falex tests                  |                         |    | Almen test—Extreme pressure (lbs.) | Timken test—Extreme pressure (lbs.) |
|----------|--------------------------|----------|---------------------------------------------------------------------------------|------------------------------|-------------------------|----|------------------------------------|-------------------------------------|
|          |                          |          |                                                                                 | Wear (125 lbs.) (mgms. loss) | Extreme pressure (lbs.) |    |                                    |                                     |
| 1-A      | 12.0                     | D        |                                                                                 | 1.0                          | 1,550                   | 15 | 15                                 |                                     |
| 18-C     | 18.0                     | D        | 0.9                                                                             | 0.7                          | 3,100                   |    |                                    |                                     |
| 18-B     | 18.0                     | D        | 0.9                                                                             | 1.1                          | 3,000                   |    | 30                                 |                                     |
| 42-A     | 20.0                     | C        | 0.9                                                                             |                              |                         | 38 |                                    |                                     |
| 42-B     | 20.0                     | C        | 0.43                                                                            |                              |                         | 38 |                                    |                                     |

In addition to the soap thickening agent, grease samples Nos. 1-A and 18-C contain 9%, by weight, white lead. The tests of Table II show that greases thickened with sulfurized metal soap thickening agents have double the extreme pressure values compared with greases thickened with unsulfurized metal soap thickening agents. Furthermore, the presence of white lead does not appear to enhance these characteristics of greases thickened with sulfurized metal soaps.

The corrosivity of greases thickened with soaps prepared by sulfurizing unsaturated free fatty acids first, then saponifying the sulfurized fatty acid to form the metal soap grease thickening agent was compared with greases thickened with sulfurized metal soaps prepared by sulfurizing the metal soaps directly.

The corrosivity of these greases was determined by immersing a polished copper strip in a 50 ml. beaker filled with the test grease at 190° F. for 100 hours. The copper strip was then washed with hexane and dried. A copper strip which was still bright after the test received a copper strip test evaluation of 10. A strip which was beginning to show a slight indication of tarnish, received an evaluation of 7. A black strip was evaluated at 3, and a strip which was black and peeling, an evaluation of 0.

Grease 7-D was prepared by first sulfurizing a mixture of fatty acids consisting of 50%, by weight, of oleic acid and 50% stearic acid by reacting 0.9 gram atom of sulfur per mole of oleic acid at 400° F. for 1 hour, then forming a lithium soap. The final grease composition contained 15.5%, by weight, of the soap thus formed plus 84.5% of a California solvent-refined paraffin base oil having a viscosity of 480 SSU at 100° F. This grease had a copper strip corrosion number of 3.

Grease 7-E was prepared by forming a lithium soap from a mixture of fatty acids consisting of 50%, by weight, of oleic acid and 50% stearic acid, then reacting the lithium soap with 0.9 gram atom of sulfur per mole of oleic acid at 400° F. for 1 hour. The final grease composition contained 15.5%, by weight, of the sulfurized lithium soap thus formed and 84.5% of a California solvent-refined paraffin base oil having a viscosity of 480 SSU at 100° F. This grease had a copper strip corrosion number of 7. The copper strip was only slightly tarnished, not corroded.

The greases of the present invention may also

contain other agents which will enhance, for example, oxidation inhibition, corrosion inhibition, etc. Other agents such as polybutenes may be added as stringiness agents, and still other agents may be added as fillers, dyes, etc.

The sulfurized metal soap thickening agents of this invention can also be used in conjunction with other thickening agents in grease compositions to inhibit wear. For example, it is known that considerable wear with steel on steel surfaces is prevalent when polysiloxane grease compositions are used as lubricants. However, when sulfurized metal soaps (e. g., sulfurized sodium oleate) are incorporated into silica thickened polysiloxane (e. g., a polymethyl phenyl siloxane) grease composition, the wear is considerably reduced.

I claim:

1. A grease composition comprising a major proportion of an oil of lubricating viscosity and from 3% to 50% of a sulfurized metal soap thickening agent obtained by reacting sulfur with a metal soap of an unsaturated fatty acid and containing from 0.25 to 1.0 atom of sulfur per double bond.

2. A grease composition comprising a major proportion of an oil of lubricating viscosity and a sulfurized metal soap thickening agent obtained by the reaction of sulfur with a soap of an unsaturated fatty acid and containing from 0.25 to 1.0 atom of sulfur per double bond, said thickening agent being present in an amount sufficient to thicken the oil to the consistency of a grease.

3. A grease composition comprising a major proportion of an oil of lubricating viscosity and from 10% to 25% of a sulfurized metal soap grease thickening agent obtained by reacting sulfur with metal soaps of unsaturated fatty acids and containing from 0.25 to 1.0 atom of sulfur per double bond.

4. A grease composition comprising a major proportion of an oil of lubricating viscosity and from 3% to 50% of a metal soap grease thickening agent, at least 5% of said soap grease thickening agent being a sulfurized metal soap thickening agent obtained by the reaction of elemental sulfur with metal soaps of unsaturated fatty acids and containing from 0.25 to 1.0 atom of sulfur per double bond.

5. A grease composition comprising a major proportion of an oil of lubricating viscosity and from 3% to 50% of a metal soap grease thickening agent, at least 15% of said soap grease thickening agent being a sulfurized metal soap thickening agent obtained by the reaction of elemental sulfur with metal soaps of unsaturated fatty acids and containing from 0.25 to 1.0 atom of sulfur per double bond.

6. A grease composition comprising a major proportion of an oil of lubricating viscosity and from 3% to 50% of a metal soap grease thickening agent, at least 5% of said metal soap grease thickening agent being a sulfurized alkali metal soap grease thickening agent obtained by the reaction of sulfur with alkali metal soaps of unsaturated fatty acids and containing from 0.25 to 1.0 atom of sulfur per double bond.

7. The grease composition of claim 6, wherein the alkali metal soap is a sodium soap.

8. A grease composition comprising a major proportion of an oil of lubricating viscosity and from 3% to 50% of a metal soap grease thickening agent, at least 5% of said metal soap grease thickening agent being a sulfurized polyvalent metal soap grease thickening agent obtained by

the reaction of sulfur with polyvalent metal soaps of unsaturated fatty acids and containing from 0.25 to 1.0 atom of sulfur per double bond.

9. A grease composition comprising a major proportion of an oil of lubricating viscosity and a metal soap grease thickening agent in an amount sufficient to thicken said oil to the consistency of a grease, said metal soap grease thickening agent containing at least 5% sulfurized metal soaps obtained by reacting elemental sulfur with metal soaps of unsaturated fatty acids having from 9 to 30 carbon atoms and from 1 to 3 double bonds per fatty acid anion, said sulfurized metal soap containing from 0.25 to 1.0 atom of sulfur per double bond.

10. A grease composition comprising a major proportion of an oil of lubricating viscosity and a metal soap grease thickening agent in an amount sufficient to thicken said oil to the consistency of a grease, said metal soap grease thickening agent containing at least 15% sulfurized metal soap obtained by reacting elemental sulfur with metal soaps of unsaturated fatty acids having 9 to 30 carbon atoms and from 1 to 3 double bonds per fatty acid anion, said sulfurized metal soap containing from 0.25 to 1.0 atom of sulfur per double bond.

11. The grease composition of claim 9, wherein the sulfurized metal soap is a sulfurized alkali metal soap of an unsaturated fatty acid.

12. The grease composition of claim 9, wherein the sulfurized metal soap is a sulfurized sodium soap of an unsaturated fatty acid.

13. The grease composition of claim 9, wherein the sulfurized metal soap is a sulfurized polyvalent metal soap.

14. The grease composition of claim 9, wherein the sulfurized metal soap is a sulfurized calcium soap.

15. The grease composition of claim 9, wherein the sulfurized metal soap is sulfurized sodium oleate.

16. The grease composition of claim 9, wherein the sulfurized metal soap is sulfurized calcium oleate.

JOSEPH A. DIXON.

References Cited in the file of this patent

UNITED STATES PATENTS

| Number    | Name       | Date          |
|-----------|------------|---------------|
| 1,957,259 | Gallsworth | May 1, 1934   |
| 2,212,189 | Brunstrum  | Aug. 20, 1940 |